

Patented Sept. 18, 1928.

1,684,401

# UNITED STATES PATENT OFFICE.

WINTHROP S. LAWRENCE, OF NEW YORK, N. Y.

## TEXTILE DYE.

No Drawing.

Application filed March 30, 1927. Serial No. 180,261.

My invention relates to products suitable for the application of dyestuffs to fabrics and refers particularly to dyestuffs in a form suitable for use as dyes and prints in the 5 coloring of fabrics and fibers.

The ordinary printing pastes and textile dyes used in the printing and dyeing of textile fabrics are not suitable for popular use, as they require expert application and involve steps of process not readily obtainable by the public.

There is a demand, however, for printing pastes and textile dyes which can be applied in the form of dyes and which can be fixed to the fiber without the necessity of extraordinary steps of process.

Among the properties essential in a practically applicable textile dye, the following may be mentioned:

20 It must be of such consistency as to flow readily from the brush; it must not spread on the fabric; must be fast to rubbing; it must be free from substances which will affect the fabric and render it weak or harsh; it must dry rapidly; should be odorless; must be non-poisonous; must penetrate the fabric and must produce results fast to washing and rubbing without steaming or similar operations.

30 I have found that all of the above-mentioned, and other, valuable attributes may be obtained in a textile dye by employing glycolic compounds as a solvent for the zinc-tannates of the basic dyestuffs.

35 By "glycolic compounds", I mean ethylene glycol, its homologues, derivatives and substitution products, among which I have found chlor-hydrin especially valuable for my product.

40 I have found that the basic-dye-zinc-tannates are soluble in glycolic compounds and that this solution can be incorporated with other chemicals to produce a textile print of most valuable properties.

45 If aqueous solutions of lakes such as are here mentioned with a solid solvent agent such as resorcin, which has been widely used in the textile dyeing industry for this purpose, were used by persons inexperienced, there would be a danger in the first washing, or by accidental wetting of the dye, of the solid solvent agent going into solution and since this solvent component is much more rapidly soluble in water than the thickening

agent, the lake would go back into solution 55 and run into the surrounding fibers causing a very undesirable smear or would be liable to stain other articles with which it was in contact.

The glycolic compounds that I prefer to use 60 are liquids, and hence, do not leave any solid residuum upon drying of the dye which, by accidental wetting, or in the first washing, would have a tendency to redissolve the coloring matter and cause running and smearing. 65

The glycolic compounds chosen have boiling points within the range of temperatures to allow of easy drying without the necessity of high temperatures.

Further, the rate of evaporation of the 70 glycolic compounds is so slow as to allow the mixture to penetrate the fabric, or fiber, before it dries.

As an example of one method of producing 75 a dye of my invention, I give the following formula, the parts indicated being by weight:—

|                                                      |    |
|------------------------------------------------------|----|
| 2 parts basic dye                                    |    |
| 6 parts tannic acid                                  | 80 |
| 3 parts zinc chloride                                |    |
| 6 parts glacial acetic acid                          |    |
| 40 parts ethylene glycol                             |    |
| 40 parts ethylene chlorhydrin aqueous solution (40%) |    |
| 70 parts gum tragacanth aqueous solution (.75%)      | 85 |

167 parts

The dye thus formed may be applied to a 90 fabric by means of a brush, or other suitable means, and is allowed to dry in the air or at a medium artificial temperature. The goods may be then washed, if desired.

In the above example, I have employed 95 both ethylene glycol and ethylene chlorhydrin, but either of these may be used alone or with small amounts of a solid solvent, such as resorcin, or phenol, which in small quantities would not be liable to produce running 100 or smearing in the hands of an inexperienced person and would be valuable as agents which would prevent bacterial or enzyme action on the gum in warm weather, in which event, however, 80 parts of ethylene glycol, or 50 105 parts of ethylene chlorhydrin may be employed.

By changing the viscosity of the solution,

it may be used for block printing, or with print rolls, and by "textile dye", I mean a mixture which may be used in the ordinary printing processes, or as a paint by brush application.

By "glycolic compound" in my claims, I mean either a single glycolic compound or a plurality of such compounds.

I do not limit myself to the particular materials, times, temperatures, quantities, or 10 steps, of procedure, as specifically described,

as these are given simply as a means for clearly describing my invention.

What I claim is:—

1. A textile dye containing a basic-dye-<sup>15</sup> zinc-tannate lake, a thickening agent and a glycolic compound.

2. A textile dye containing a basic-dye-zinc-tannate lake, a thickening agent and chlorhydrin.

WINTHROP S. LAWRENCE.